

Oct. 3, 1933.

J. B. NEAL

1,928,699

METHOD OF MAKING MINERAL WOOL MIXTURE

Original Filed July 27, 1927



INVENTOR  
JAMES B. NEAL

by Robert Cushman Woodberry  
ATT'Y

## UNITED STATES PATENT OFFICE

1,928,699

## METHOD OF MAKING MINERAL WOOL MIXTURE

James B. Neal, Lockport, N. Y., assignor, by  
mesne assignments, to Johns-Manville Corpora-  
tion, New York, N. Y., a corporation of New  
York

Original application July 27, 1927, Serial No.  
208,810. Divided and this application October  
6, 1931. Serial No. 567,203

## 3 Claims. (Cl. 154—28)

This invention relates to the manufacture of  
heat insulating materials comprising mineral  
wool or rock wool filaments and sustaining or  
strengthening fibres, such as asbestos; one object  
5 of the invention being the provision of a durable,  
fire-resisting, heat insulating material, adapted  
to such uses as the insulation of ice-houses, cold  
storage rooms, steam pipes, etc.

The filaments of mineral wool are vitreous, and  
10 though to a sensible degree flexible and elastic,  
are nevertheless brittle and tend to break up into  
small fragments forming a coarse dust; this de-  
terioration of the product is not only incident to  
handling but also occurs after it has been placed  
15 in wall-spaces for heat insulation purposes, as a  
result of jarring and vibrations to which all struc-  
tures are subjected more or less.

By the invention herein described, sustaining  
or reinforcing fibres, inherently tougher than  
20 mineral wool filaments, are intermixed with the  
mineral wool filaments with substantially uni-  
form distribution; the mixture is effected without  
subjecting the mineral wool to mechanical han-  
dling, and preferably before the mineral wool  
25 fibres or filaments have settled for the first time  
after their formation by the usual pneumatic  
means. Once the mineral wool filaments have  
settled on each other to form a loose, tangled ag-  
gregate, they can not thereafter be freely sep-  
30 arated or dispersed as individual filaments and  
therefore no fully satisfactory approximation to  
a uniform distribution of other fibres through the  
aggregate is possible. This invention in its aspect  
of method and in its preferred mode is charac-  
35 terized by the introduction of dispersed sustain-  
ing fibres among the mineral wool fibres by  
pneumatic means, while both the mineral wool  
filaments and sustaining fibres are held suspen-  
ed and dispersed in pneumatic currents, which  
40 by their intermixture and confluence cause  
mutual intermixture of the two kinds of fibre  
preferably before the mineral wool fibres have  
settled out of the stream of air and water vapor  
45 which bears them from their point of origin,  
where the molten slag or rock is blown into fila-  
ments by the steam jet in the well known man-  
ner. Other aspects and features of the inven-  
tion will transpire from the description herein  
50 below.

The physical conditions which characterize  
this invention might measurably be obtained by  
imperfect dispersion of mineral wool fibres by  
pneumatic means applied thereto after their  
55 initial settlement and mixture therewith, while

in such state of dispersion as might be thus  
effected, of dispersed sustaining fibres.

The material preferred, for imparting strength  
and durability to a fibrous mass predominantly  
consisting of mineral wool, is asbestos fibre, which  
is, like the mineral wool itself, incombustible.

The method will be explained by reference to  
the drawing hereto annexed, which represents  
an apparatus by which the method may be prac-  
ticed and the product obtained. In this draw-  
ing, A represents a cupola furnace, in which the  
rock or slag material is fused, B the tap from  
which fused rock is drawn to flow in a thin stream,  
C the nozzle from which a steam blast issues, to  
disrupt the stream of melted rock and draw it  
out into fine filaments; D the wool-bin, D' the  
aperture in the side of the wool-bin through  
which the gaseous stream, bearing dispersed rock  
filaments, is blown, K a conveyor on which the  
rock wool W settles and is conveyed out of the  
wool-bin through the aperture D' therein.

The travel of the conveyor is adjusted so that  
the fibrous material is removed from the wool-  
bin at the same rate that it is delivered in; this  
prevents accumulation of fibre in the bin and con-  
sequent reduction of the free air space therein,  
and thus preserves constant the conditions under  
which the two classes of fibres are mixed together,  
ensuring a uniform mixed product.

To accomplish this object with a minimum of  
fracture of the mineral wool fibres, pneumatic, as  
distinguished from mechanical means for pro-  
ducing a state of dispersion of the fibres, are em-  
ployed, particularly with respect to the mineral  
wool fibres. The sustaining fibres, as of asbestos,  
being mechanically stronger than the mineral  
wool fibres, may, and normally will, be subjected  
to mechanical dispersion in preparation for in-  
terspersion with the mineral wool fibres.

Furthermore, as the mineral wool fibres are,  
as an incident to their mode of formation, ini-  
tially borne by and suspended in a state of dis-  
persion in, a pneumatic stream, the object of  
mixture with sustaining fibres with a minimum  
of damage to the mineral wool fibres will best be  
100 served by effecting this mixture while the min-  
eral wool fibres are in their initial stage of dis-  
persion, and before their first settlement into a  
mass of tangled filaments.

Referring again to the drawing hereto an-  
nexed:

P represents an air-pipe leading from an in-  
take G to a fan-blower F. The intake G is pref-  
erably from the interior of the wool-bin D, so  
that floating fibres will be drawn to the blower 110

and so that the introduction of the asbestos-fibre bearing blast will not lower the temperature or increase the pneumatic pressure in the wool-bin. L represents a feed box for introducing asbestos fibre to the intake pipe P. H represents an air blast pipe, leading from the blower E to the delivery nozzle I, within the wool-bin, which is so directed as to deliver an air stream in which asbestos fibres are dispersed and borne, into confluence with the pneumatic stream which bears dispersed mineral wool fibres W. The confluence of these two fibre-bearing streams produces eddies which effect a substantially uniform mutual intermixture of the two types of fibres, while the mineral wool fibres are, so to speak, in their nascent stage, so that, as the mixed fibres settle on the conveyor K in a mixture M, the mineral wool fibres are matted loosely for the first time, and settle with the dispersed asbestos fibre uniformly distributed through the mass. Thus the mixture of sustaining fibres with mineral wool fibres is effected with no more mechanical injury to individual mineral wool fibres than is incidental to the primary settling of the said fibres.

While, in the fibre-mixture thus produced small tufts of asbestos fibre will be perceptible, these are accounted for by the unavoidable imperfections in the dispersion of the asbestos fibres; a large proportion of the asbestos fibres is distributed as single fibres or very small aggregates, throughout the mass of mineral wool fibre.

The proportion of mineral wool to asbestos may be varied to suit the purposes of the manufacturer. The normal variations will lie, probably between 20% and 50% of asbestos, to 80% and 50% mineral wool fibre.

The uniformity of distribution of sustaining fibres through a mass of mineral wool fibres, produced by the above-described method minimizes

the liability of the matted fibres to be broken and crushed in handling and thus preserves the heat-insulating efficiency of the fibre mass. The adjusted rate of travel of the conveyor belt K contributes to this end, since the continuous removal of the fibre mixture from the wool-bin permits its accumulation into a deep mass and dispenses with intermittent mechanical removal of such masses. Moreover, as the mixture of the two classes of fibres is effected by pneumatic currents and eddies, it is important to maintain unchanged the volume and shape of the space within which such currents and eddies perform their function; this is provided for by the correspondence between the rates of introduction and withdrawal of fibre material.

I claim:

1. Method of making a mixture of mineral wool filaments and sustaining fibers, characterized by feeding fused rock into a fluid stream to form mineral filaments in fluid suspension and directing pneumatically suspended and dispersed supporting fibers between the suspended filaments, and then allowing the resulting mixture to settle. 80

2. Method of making a mixture of mineral wool filaments and sustaining fibers, characterized by blowing fused rock into the air to form dispersed mineral filaments, directing sustaining fibers upon a pneumatic stream into intermingled relation with the filaments while still in the air, and permitting the resulting mixture to settle. 85

3. Method of making a mixture of mineral wool filaments and sustaining fibres, characterized by employing a fluid stream directed into the air to form filaments from fused rock, employing a confluent pneumatic stream to bear sustaining fibers so that the fibers are mixed with the mineral filaments while the latter are still in the air, and allowing the filaments and fibers to settle as thus mixed. 90

JAMES B. NEAL.